

April 10, 1928.

1,665,844

J. J. CONLIN

METHOD OF PURIFYING METALS

Filed April 6, 1927



Inventor:  
John J. Conlin,

by *Myron S. Linn*  
His Attorney.

## UNITED STATES PATENT OFFICE.

JOHN J. CONLIN, OF SCHENECTADY, NEW YORK, ASSIGNOR TO GENERAL ELECTRIC COMPANY, A CORPORATION OF NEW YORK.

## METHOD OF PURIFYING METALS.

Application filed April 6, 1927. Serial No. 181,543.

The present invention relates to the purification of metals and more particularly to the purification of metals of the alkali or alkaline earth groups. Certain of these metals, particularly calcium and magnesium, are frequently employed as "getters" in vacuum tube construction. They are readily oxidizable and normally contain a considerable percentage of impurities, usually in the form of salts, which it is desirable to remove before the metal is introduced into vacuum tubes.

It is one of the objects of the present invention to provide a simple and inexpensive process for the removal of such included salts. It is a further object of the invention to provide a method for forming an alloy of a plurality of such metals at the same time that the impurities are removed there-

from. The novel features which I believe to be characteristic of my invention are set forth in the appended claims. My invention itself, however, will best be understood from reference to the following specification when taken in connection with the accompanying drawing in which the single figure shows a cross section of an apparatus whereby my invention may be carried into effect.

Referring to the drawing, I have indicated at 1 a suitable furnace having a burner 2 located adjacent the lower end thereof, the burner being supplied with gas and air through pipes 3 and 4 respectively. An open metallic container 5 partially filled with a suitable salt, such as calcium chloride, is mounted in the furnace so that the flames from the burner may be directed around the lower end thereof. Calcium is inserted into a steel tube 6 which is about  $2\frac{1}{2}$  inches in diameter and 9 inches long. The upper end of the tube is closed by a plug 7 and provided with an elongated handle 8. A metal plug 9 approximately  $\frac{1}{2}$  inch in thickness and having a small opening 10 is detachably secured by a bolt or screws 11 at the lower end of the tube.

In operation the calcium chloride is gradually heated up to a temperature of about  $900^{\circ}$  C. When the temperature has been raised to about  $800^{\circ}$  C., the steel tube 6 containing the calcium is immersed to a slight extent in the salt and as the temperature of the latter is raised the tube is gradually lowered into the salt. When the upper tem-

perature limit  $900^{\circ}$  C. has been reached the tube is entirely submerged and held in this position for about five minutes. The entire operation consumes approximately twenty minutes. Substantially pure calcium floats 60 to the top of the tube, while the calcium salts sink to the bottom. There is a sharp line of demarcation between the calcium and the salts and the latter may be easily separated from the calcium by removing plug 9 and 65 cutting the tube 6 lengthwise.

The opening 10 acts as a safety valve and prevents the pressure in tube 6 from rising too high. Although a small amount of calcium salt enters tube 6 through this opening, this action does not interfere with the operation of the process since the salt which enters remains at the bottom of the tube.

The same process may be employed with other oxidizable metals, such as magnesium. 75 Furthermore, other salts than calcium chloride may be employed if desired, the main consideration for such salts being that they should not be volatile at  $900^{\circ}$  C. and should not react with the metal which it is desired 80 to purify.

The process may also be employed to simultaneously purify a plurality of metals and to form an alloy of the metals at the same time that the impurities are removed. 85 For example, if magnesium is placed in the upper part of tube 6 and calcium in the lower part, and the tube then immersed in molten calcium chloride as above described, the included salts in the calcium and magnesium 90 will sink to the bottom of the tube while the magnesium and calcium will rise above the salts and form a substantially pure alloy that is particularly adaptable for use as a "getter" in vacuum tubes.

What I claim as new and desire to secure by Letters Patent of the United States, is:

1. The method of purifying a readily oxidizable metal which comprises placing the metal in a container provided with a 100 vent and submerging the container in molten material which does not react with said metal and which has a temperature sufficiently high to cause separation of the metal and impurities contained therein.

2. The method of treating a readily oxidizable metal which comprises placing it in a rigid container having an opening in the lower portion thereof and immersing the container in a molten salt which does not 110

react with said metal and which has a temperature sufficiently high to cause separation of the metal and impurities contained therein.

3. The method of purifying a readily oxidizable metal which comprises placing the metal in a container having an opening in the lower end thereof and immersing the container in a salt which does not react with 10 the said metal and which has a temperature sufficiently high to cause separation of the metal and impurities contained therein.

4. The method of preparing a substantially pure alloy which comprises placing the 15 metals comprising the alloy in a container having a vent therein and submerging the

container in a molten salt which does not react with said metals and which has a temperature sufficiently high to cause separation of the metal and impurities contained 20 therein.

5. The method of preparing a substantially pure alloy of alkaline earth metals which comprises placing the metals in a container having an opening in the lower 25 end thereof and immersing the container for a period of at least five minutes in a salt which does not react with said metals and which has a temperature of about 900° C.

In witness whereof, I have hereunto set 30 my hand this 5th day of April, 1927.

JOHN J. CONLIN.